

March 20, 1945.

A. F. TURNER

2,371,786

METHOD OF PRODUCING ABRASIVE

Filed May 31, 1943



ARTHUR F. TURNER  
INVENTOR.

BY *J.A. Collested*  
*G.J. Amyth*

ATTORNEYS

## UNITED STATES PATENT OFFICE

2,371,786

## METHOD OF PRODUCING ABRASIVES

Arthur F. Turner, Brighton, N. Y., assignor to  
 Bausch & Lomb Optical Company, Rochester,  
 N. Y., a corporation of New York

Application May 31, 1943, Serial No. 489,162

4 Claims. (Cl. 51—293)

This invention relates to abrasive and polishing materials and the apparatus and method of forming the same.

In certain industries, such as the optical industry, where it is highly essential that the abrasive or polishing materials used during the final grinding and polishing operations be extremely fine, considerable difficulty has been heretofore experienced in grinding the materials to the fineness desired. Not only has considerable difficulty been experienced in grinding the materials to the fineness necessary, but it has been also difficult to make certain that no particles larger than the maximum to be tolerated will be present in the finished material. Although a number of screening and separating processes are usually performed before the material is considered ready for use, there is always the danger that excessively large grains may be present in the material. It will be appreciated that several or even one excessively large grain can destroy a highly polished surface.

The present invention avoids the difficulties of the prior art in that the abrading material is not broken up into extremely fine particles but is actually formed at the outset of particles having a controlled desirable thickness. This is accomplished by forming the final product by a high vacuum thermal evaporation process where-in the vapors of the abrasive-forming material are allowed to condense on a suitable support.

As the thickness of the film formed by the distilled material on the support can be controlled, the thickness of the abrasive or polishing flakes formed by removing the film from the support can also be controlled. Thus the process of the present invention is the reverse of the ordinary process of forming fine abrasives where-in the different size particles must be separated out by sedimentation or an equivalent process.

In the embodiment of the invention now preferred, the support is formed with a substantially spherical surface and is held in an inverted position over the material to be evaporated. The support is preferably formed of a transparent material such as glass so that the film being deposited can be examined during the evaporation process.

The material to be evaporated is held by a crucible heated from above by a heating element formed of a flat tungsten spiral and to secure an even deposit from such a flat source it is spaced downwardly from the vertex of the support a distance equal to twice the radius of the spherical surface of the support.

A feature of the present invention, therefore, is the ability to prepare a fine polishing or abrading material of a definite and uniform thickness. Thus it is possible to form such material free of any large particles which might cause scratching or stripping.

If desired, the support on which the vapors are condensed can be used as a storage chamber after the evaporation process has been completed by sealing the film-carrying surface or two supports can be brought together to form a single storage container and the line of jointure sealed to prevent foreign matter from becoming mingled with the abrasive held by the storage container.

If it is desired to store the material of the present invention ready for use the material can be removed from the interior of the support and stored in a medium such as water until used.

Other features and advantages of the present invention will more clearly appear from the following description taken in conjunction with the accompanying drawing in which:

Fig. 1 is a sectional view partly in elevation of the apparatus of the present invention.

Fig. 2 is a sectional view partly in elevation of a modified form of the apparatus of the present invention.

The apparatus of the present invention, referring now to the drawing, comprises a suitable base plate 10 which supports an evacuable container shown here as a bell jar 11 of glass or other material. A vacuum tight seal is formed between the lower edge of the bell jar 11 and the base plate 10 by any suitable sealing means 12. The bell jar 11 is connected by some conventional means such as the pipe 13 to a high vacuum pump shown here diagrammatically at 14.

Mounted on the base plate 10 are a plurality of stanchions 15 supporting a carrier 16 on which is placed a support 17, preferably formed of some transparent material such as glass. In the illustrated embodiment of the invention, the support has been shown as substantially hemispherical in shape although it is to be understood that the support can take other forms having spherical or substantially spherical undersurfaces. The carrier 16 is formed with a large central opening 18 having a diameter equal to or greater than the diameter of the mouth of the support 17.

The material to be evaporated is supported within a crucible 19 mounted above the base plate 10 by any suitable support 20. The material to be evaporated is heated from above by a

heating element 21 comprising a flat spiral of tungsten wire supported above the crucible 19 by small rods 22 of current conducting material carried by suitable bushings 23 of insulating material mounted in apertures in the base plate 18. The heating element 21 is connected through the posts 22 and lead-in conductors 24 to a source of current, not shown.

In carrying out the process of the present invention after the apparatus has been set up as disclosed in Fig. 1, the bell jar is sealed and evacuated by means of the pump 14. After the bell jar has been evacuated and the pressure reduced therein to the minimum desired, the heating element 21 is energized to heat the material disposed in the crucible to the evaporating temperature thereof, whereafter the vapors of the material will travel toward and condense on the under surface of the hemispherical support 17. This process would be carried on until the material held by the crucible 19 was completely evaporated or until the film formed by the condensed vapors on the undersurface of the support 17 had reached the desired thickness.

It has been found that a uniform deposit may be obtained from the relatively large flat source formed by the exposed surface of the material held by the crucible 19 if the latter is so mounted that the surface of the material is substantially tangent to the sphere of which the spherical undersurface of the support forms a part. This relationship can be brought about by mounting the crucible relative to the support so that the surface of material is spaced downwardly from the vertex of the surface to be coated a distance equal to substantially twice the radius of curvature of the surface of the support. That the thickness of the film deposited is uniform will be evident by the uniformity of the interference colors over the entire surface on which the film is being deposited.

It has been found that the deposited film generally begins to loosen and crack away from the surface of the support when the film reaches substantially one micron in thickness. The evaporation is continued, however, beyond this point and preferably until the film reaches a thickness of approximately two to three microns.

The thickness can be checked by counting interference bands on a small section of the support which is shadowed from the direct molecular beam from the material being evaporated by a small shield 25 supported adjacent a portion of the undersurface of the support 17 by a bracket 26 carried by one of the stanchions 15. It has been found that the deposit formed in the shadow of the shield can be built up to a much greater thickness without the film cracking and pulling loose from the supporting surface. The interference bands are counted adjacent the edge of the shadow where the thickness of the film deposited is nearly that of the film formed on the remainder of the undersurface of the support.

After the film has reached the desired thickness the bell jar can be removed from the base plate 18 and the support carefully removed from the carrier 16. Upon removal of the support from the bell jar 11 the deposit can be brushed off the former and stored in a liquid until ready for use on the polishing lap. If desired, however, the abrasive material thus formed may be stored within the support by sealing the mouth thereof by any suitable means or two coated supports may be placed together with the line of juncture

sealed and the abrasive material stored in the storage container so formed until ready for use.

The abrasive or polishing flakes formed when the film is removed from the surface of the support will vary in area but will never have a thickness greater than the controllable thickness of the deposited film. The lateral dimensions of the flakes will change as they are broken up during the polishing operation but as the thickness of the flake can be controlled by the film forming operations, polishing material can be formed which is absolutely free of any particles having a thickness greater than a predetermined one and which might scratch or otherwise mar the surface being polished.

Any material which can be evaporated and which has abrasive or polishing qualities can be used to form the material of the present invention. I have found magnesium fluoride and sodium aluminum fluoride to be readily evaporable and both form excellent polishing materials when the finished material is formed by the process of the present invention. Abrasive materials of the two fluorides mentioned have been very successfully used for polishing calcite. Stannic oxide, often used for polishing steel and like metals, has been found to evaporate readily and extremely fine polished metallic surfaces have been attained by using distilled material formed by evaporating this oxide.

In polishing material heretofore used, it has usually been found desirable to use a polishing medium which will have a higher melting point than that of the substance being polished and it appears that this will also be true of the material of the present invention.

In the broadest aspects of the present invention, any support can be used to collect the vapors of the material evaporated and the bell jar itself could, if desired, be used as the support on which the film would condense. Furthermore, a flat support could be used as long as the thickness of the distilled material was not allowed to exceed the maximum thickness which could be tolerated. In Fig. 2, there is shown a modified form of the support 17. In this form, the support comprises a hollow spherical member 30 having an opening 31 in the wall thereof, just large enough to permit a crucible 32 and a heating element 33 with its support to be placed therein. In this form of the present invention, the member 30 can be either placed in an evacuable container such as the bell jar 11 or the opening 31 sealed and the member 30 itself evacuated.

It will be noted that the crucible 32 is again spaced downwardly from the vertex of the inner surface of the member 30 a distance substantially equal to the diameter of the same and that the inner surface of the member if extended would be substantially tangent to the surface of the material held within the crucible 32.

The opening 31 can be sealed after the completion of the evaporation process so that the distilled material may be stored therein until it is to be used. To permit the opening 31 to be quite easily sealed, it may be formed with a neck portion 34 and a suitable stopple placed in the bore of the neck portion.

It is to be understood that while the preferred embodiments of the present invention have been described and illustrated herein, the invention is not to be limited thereby but is susceptible of changes in form and detail within the scope of the appended claims.

I claim:

1. The method of forming an abrasive and polishing compound comprising the steps of evaporating an abrasive-forming material in an evacuated space in close proximity to a surface of a transparent body so that vapors from said material may condense thereon; discontinuing the evaporation of said material after light ray interference bands indicative of a desired thickness of distilled material are discernible through said transparent body; and thereafter removing said distilled material from said surface.

2. In the method of forming an abrasive and polishing compound material the steps of evaporating an abrasive-forming material in an evacuated container; collecting the vapors of said material by mounting a support adjacent to said material having a concave surface on which said vapors may condense; removing said support from said container; and placing a seal over said surface to prevent foreign matter from mingling with the condensed material until said material is to be removed from the surface and used.

3. A method of preparing an abrasive material having a predetermined flake thickness which

comprises the steps of evaporating the abrasive material in an evacuated container, condensing the vapor on a support, and determining the thickness of the layer of the material deposited on the support by observing interference bands caused by light rays which strike the condensed layer of material on the support whereby the abrasive flakes may be held to a predetermined thickness, and thereafter removing the material from the support.

4. A method of preparing an abrasive material having a predetermined maximum flake thickness which comprises the steps of evaporating the abrasive material in an evacuated chamber, condensing the vapors on a surface of a transparent support, and determining the thickness of the layer of material deposited on said support by observing through the support the interference bands caused by light rays which strike the layer of material whereby the abrasive flakes may be held to a predetermined thickness, and thereafter removing the abrasive material from the support.

ARTHUR F. TURNER.